

# UNITED STATES PATENT OFFICE.

FREDERICK LAIST AND JAMES ORR ELTON, OF ANACONDA, MONTANA, ASSIGNORS TO ANACONDA COPPER MINING COMPANY, OF ANACONDA, MONTANA, A CORPORATION OF MONTANA.

## METHOD OF PURIFYING ZINC-BEARING SOLUTIONS.

1,255,435.

Specification of Letters Patent.

Patented Feb. 5, 1918.

No Drawing.

Application filed June 16, 1916. Serial No. 104,083.

To all whom it may concern:

Be it known that we, FREDERICK LAIST and JAMES ORR ELTON, citizens of the United States, residing at Anaconda, in the county of Deerlodge and State of Montana, have invented certain new and useful Improvements in Methods of Purifying Zinc-Bearing Solutions, of which the following is a specification.

10 Zinc-bearing solutions, such for example as those prepared by leaching calcined zinc ores with dilute sulfuric acid, are readily purified from iron, and from a part at least of their content of arsenic and antimony. 15 This may be accomplished for example by effecting a complete oxidation of the iron salts in the solution, and then precipitating the same by such basic reagents as zinc oxide or lime; under these conditions arsenic and 20 antimony are largely precipitated with the ferric iron, as disclosed for example in the prior patents to Laist and Frick, Numbers 1,167,700 and 1,167,701. The resulting solutions however, usually carry other impurities, notably copper and cadmium, the complete elimination of which offers considerable difficulties. On the other hand such 25 complete elimination is a practical necessity, inasmuch as the presence of these 30 metals even in very small proportions tends to reduce the current efficiency in the subsequent electrolytic deposition of zinc, and tends also to a poorer quality of deposit.

We have found that zinc sponge, prepared by electrolytic precipitation from zinc salt solutions, is a highly efficient agent for the treatment of impure zinc-bearing solutions, especially for the separation therefrom of traces of copper and cadmium. As 40 hereinafter pointed out this zinc sponge may be prepared by electrolyzing pure zinc salt solutions, in which case a pure zinc sponge is obtained; or it may be prepared by electrolysis of the solutions which are 45 to be purified, in which case a double result is achieved, to wit, the solutions from which the sponge is precipitated are purified either wholly or in part; and zinc sponge is obtained in suitable condition for the treatment 50 of the same or other zinc-bearing solutions.

In either case zinc anodes are used, which are electrolytically dissolved, thereby maintaining normal conditions in the electrolyte

as regards acidity and concentration. According to the voltage and current density employed, the zinc sponge may separate out upon the cathodes, or upon the bottom of the cell, or it may remain suspended in the electrolyte; or it may appear in any two or all of these conditions. Our invention is therefore not restricted to the employment of any specific electrical conditions, although we have found it desirable to use voltages between 0.5 and 2.3, the corresponding current densities lying between 2 and 30 amperes, per square centimeter of active electrode surface. These conditions may, however, be considerably varied, provided only a fine spongy deposit is obtained. At the lower voltages mentioned above more of the sponge tends to collect upon the bottom of the cell, where it is immediately available for use.

This sponge may be directly used without drying, the solution to be purified being thoroughly agitated therewith, after which the excess of zinc is permitted to settle out from the solution, and is reused so long as it retains its efficiency. When it becomes too high in copper and cadmium, it may be refined in any known manner for the recovery of its components.

Or the wet sponge may be dried under strictly non-oxidizing conditions, for example in a current of any inert gas, or *in vacuo*, after which it is available for use in place of the regular furnace product, being superior thereto as a precipitant.

A highly advantageous mode of operation in accordance with this invention is as follows:—

Impure zinc-bearing solutions, as for example zinc sulfate solutions from which iron, arsenic and antimony have been separated as noted above, are caused to flow rapidly through an electrolytic cell having anodes of zinc, the cathodes being either zinc or any other suitable conductive material, the electrical conditions being controlled to effect the deposition of zinc as sponge as specified above. If the rate of flow of the solution is sufficiently slow, its complete purification may be accomplished in the course of its passage through the electrolytic cell, and the sponge is then available for the treatment either of other solutions or of other portions of the same solution. If

however, the flow is maintained at a rate in excess of that at which complete purification is obtainable, the precipitated zinc sponge may be carried forward into an agitator in the line of flow of the solution from the electrolytic cell, and is used to complete the purification of this solution. By proceeding in this way we secure a rapid and substantially complete purification of the solution with a minimum use of zinc and a minimum expenditure of power. In this operation we prefer to employ voltages of a comparatively low range, preferably below those required for the deposition of zinc with insoluble anodes.

We prefer to employ one, or preferably more, combination agitating and settling tanks operating as follows: The tanks are charged with the zinc sponge, or with zinc dust or sludge from any other source if such be available, in large excess of the amount actually required for the purification of the solution. In these tanks the solution is thoroughly agitated with the zinc until the purification is complete or has proceeded as far as is necessary, after which the agitator is stopped and the excess of zinc, together with the separated impurities is permitted to subside. The clear solution is now drawn off, and the above operation repeated with further quantities of solution to be purified, until the zinc is exhausted or its efficiency lost. By proceeding in this way the usual heavy wastage of zinc is avoided. Any suitable type of apparatus may be used for this purpose, as for example a tank of the ordinary Pachuca type, provided with an efficient stirrer, and with a draw-off above the conical bottom for the clear solution. Such apparatus is well known in the art and need not be further described.

A further modification of the invention consists in subjecting the zinc-bearing solution which is to be purified, to the action of zinc anodes, the current conditions being so regulated that little or no zinc is deposited in the form of sponge or otherwise, the electrodeposition being substantially or wholly restricted to the more electro-nega-

tive components of the solution, usually including copper and cadmium. In this way, operating with low current densities, the solution may be more or less completely purified depending upon its rate of flow through the cells. The precipitated impurities will settle upon the bottom of the cell as a sludge, deposit upon the cathodes, or be held in suspension in the electrolyte from which they may be removed by any appropriate clarifying means, as by filtration or settling.

We claim:—

1. In a process of purifying zinc-bearing solutions, the step which consists in subjecting the impure solutions to the action of electrolytically deposited zinc sponge.

2. A process of purifying zinc-bearing solutions and recovering metallic zinc, which consists in passing an electric current through the impure solution from anode surfaces of zinc to purify the solution, and thereafter electrodepositing zinc from the purified solution.

3. A process of purifying zinc-bearing solutions, which consists in passing an electric current through the impure solution from anode surfaces of zinc under conditions to form a deposit of zinc sponge.

4. A process of purifying zinc-bearing solutions, which consists in passing an electric current through the impure solution from anode surfaces of zinc under conditions to form a deposit of zinc sponge, and subjecting the partially purified solution to agitation in the presence of the zinc sponge thus produced.

5. A process of purifying zinc-bearing solutions, which consists in passing an electric current through the impure solution from an anode surface of zinc, and thereafter agitating the partially purified solution in the presence of finely divided zinc to complete the purification.

In testimony whereof, we affix our signatures.

FREDERICK LAIST.  
JAMES ORR ELTON.